# EUROPEAN PATENT SPECIFICATION

(11) **EP 1 796 860 B1**
(45) Date of publication and mention of the grant of the patent: **06.08.2008**
(21) Application number: 05785271.7
(22) Date of filing: 08.09.2005
(51) Int. Cl.: B21D 13/02, B21D 13/04, B21D 22/02, C22C 45/02, B21D 37/20

(54) **MODIFYING SURFACES OF WORK-PIECES AND FORMING TOOLS**
MODIFIKATIONSFLÄCHEN VON WERKSTÜCKEN UND FORMWERKZEUG
MODIFICATION DE SURFACES DE PIECES A USINER ET OUTILS DE FORMAGE

(30) Priority: 20.09.2004 EP 04405604
(43) Date of publication of application: 20.06.2007
(73) Proprietor: Alcan Technology & Management Ltd., 8212 Neuhausen am Rheinfall (CH)
(72) Inventor: HOTZ, Walter, CH-8222 Beringen (CH)
(86) International application number: PCT/EP2005/009630
(87) International publication number: WO 2006/032369

(56) References cited:
- US-A1- 2002 018 908
- PATENT ABSTRACTS OF JAPAN vol. 1999, no. 01, 29 January 1999 (1999-01-29) -& JP 10 265917 A (INOUE AKIHISA), 6 October 1998 (1998-10-06)
- PATENT ABSTRACTS OF JAPAN vol. 007, no. 031 (M-192), 8 February 1983 (1983-02-08) -& JP 57 187127 A (NISSAN MOTOR LTD), 17 November 1982 (1982-11-17)

## Description

The present invention relates to a forming tool, a method of modifying the surface of a work-piece wherein at least one surface of the work-piece comes into contact with the structured surface of a forming tool at least once and a method of structuring the outer surface of a forming tool, according to the preambles of claims 1, 15 and 21 respectively (see for example JP-A-10265917).

In the materials processing industries there are many types of forming operation. In the metals industry forming operations can include, for example: press forming, where the work-piece to be formed takes the shape imposed by a punch and a die; drawing, where a work-piece in the form of a flat blank of sheet is formed into a cup shape by forcing a punch against the central portion of the blank as it rests on a die ring; coining, where a work-piece is squeezed between dies and is deformed such that the details of its final form and surface appearance are defined by the shape and surface of the dies; stretch forming, where a sheet blank work-piece is formed over a form block of the required shape with the work-piece under tension; drop hammer processing; stamping, which is similar to coining; embossing, which is generally the making of shallow impressions in the surface of a work-piece by compression between two die pieces under a relatively low load; texturing, which is similar to embossing but where more load is applied leading to more deformation into the bulk work-piece; rolling, where work-pieces in the form of sheets are pressed between two rotating cylindrical rolls; and cold roll forming, where the rotating rolls are shaped such that the sheet work-piece is formed into desired shapes of uniform cross-section.

A work-piece is a body of indeterminate size and shape. For example a block of metal or plastic is a work-piece and so are pre-formed articles for use as vehicle panels. Sheet, plate and foil, both in continuous form and in the form of cut pieces, are further examples of work-pieces. In one form of the invention the work-piece is preferably rolled sheet or strip and is more preferably rolled sheet or strip of aluminium and aluminium-based alloys.

In this invention a structured surface is meant to be where the surface is not intended to be smooth. Of course most surfaces are not perfectly smooth, but it will be readily understand what is covered by the meaning of a structured surface if it is defined as one possessing deliberate roughness, patterns, protuberances, depressions, ridges and troughs or engraving-like features, such features to be transmitted to the surface of the work-piece such that the work-piece surface is also not smooth.

Typically forming operations like this are applied to metals, in particular metals based on iron, aluminium or copper as the main constituent, but they may also be applied to plastic materials. In some cases a forming method like embossing can be applied to paper-based materials.

During such forming operations, the appearance of the surface of the work-piece which was in contact with the forming surface of the forming tool after forming is typically the same as or similar to the surface appearance of forming surface of the forming tool. The surface on the work-piece may not be an exact replica of the surface of the forming tool because various factors like the amount of load applied through the forming tool or the physical properties of the material of the work-piece have an influence on the extent of deformation. It is routine practice to adjust forming conditions to take account of such factors. Often the surface of the forming tool may be exaggerated in order to ensure the final surface on the work-piece is produced.

There are also many situations where the surface of a work-piece is desirably modified in order to bring about specific benefits. The surfaces of work-pieces may be modified for purely decorative reasons. Examples are where a coining operation is used to produce coins, buttons or medals to specific designs. Other examples are where a metallic sheet work-piece is treated such that it has a certain range of roughness across the surface in order to mask any defects that might be present after a rolling operation. This is often done in order to give a uniform appearance to the final product. The surface of a work-piece may also be modified in order to attain desirable physical characteristics with the aim of improving the performance of an article in a specific application, where that performance depends strongly on the surface characteristics of the work-piece.

When modifying the surface of flat sheet the forming tools may have on their surface a textured surface prepared by one of a variety of methods. Such known methods include EDT texturing, sand blasting or shot peening, mechanical brushing, structured Cr deposition (also known as Topocrom), and so on. These methods result in a working surface which is stochastic in nature and after rolling this surface structure is substantially transferred to the surface of the work-piece. Other known methods include laser beam or electron beam texturing and these can produce a deterministic structure. A deterministic structure would show a pattern, or would be one where a specific design is present and could include, for example, an imprint of wording or an imprint of a trade mark. Deterministic structures can also be a drawing or a parabolic topography or a grating. In the case of multiple pass embossing, deterministic structures can lead to interference effects whilst stochastic structures generally will not.

In work rolls used for forming metal sheet by rolling, a deterministic structure could be imparted into the surface of the work roll by a machining operation, but this would be expensive and such work rolls have a limited life whereafter they need to be refurbished or re-machined, operations which can be expensive and time consuming. Furthermore, the quality of indentation of the deterministic structure into the surface of the work-piece may deteriorate over time due to wear of the forming surface of the forming tool leading to variable quality in the final product over long production runs.

Deterministic structures are more readily and more commonly produced in the surfaces of work-pieces using methods such as coining, stamping or press forming where it is common to machine the desired design into the surface of the die or punch.

In most of the forming operations mentioned above there is eventually a need to replace dies, punches, rolls and other tools used for forming, or to refurbish the same. This, of course, depends on the material from which the work-piece is made with harder work-pieces leading to faster wear of forming tools than softer work-pieces.

The life of a forming tool is often extended by adding a protective layer to that surface of the forming tool that comes into contact with the work-piece. In forming operations using dies and punches, such protective coatings are usually deposited onto the working surface of the tool without any subsequent profiling step, i.e. they are applied in such a way that the shape required is still derived from the shape defined by the main body and profile of the forming tool itself.

In metal rolling, particularly aluminium rolling, a steel work roll is often protected with a chromium layer to extend the life of the working roll. Typically such work rolls have their surfaces ground flat because the intended use of such rolls is merely to reduce the thickness of plate, sheet or foil through a mill. When the main purpose is thickness reduction a major consideration is to obtain as smooth a surface as possible on the rolled sheet at the end of a series of rolling passes.

However, where a structured surface is desired, it is possible to modify the structure of the chromium layer. It is also possible to structure the underlying steel of the work roll and deposit a layer of chromium over the roll. For modifying the structure of the chromium layer itself, one known technique involves applying a photosensitive film to the chromium layer. A pulsed laser can be scanned across the surface and, where it scans, the heat of the laser polymerises the film. The unpolymerised film can be washed away exposing chromium underneath. The exposed chromium can be etched away to a required depth whilst the chromium under the polymerised masking remains as it was. This leads to the creation of an irregular roll surface with the final form of the roll surface dictated by the path of the laser.

These protective coatings, whilst beneficial in many respects, have the disadvantage that it is not possible to provide them with very fine detailed designs of a deterministic nature. For example, the chromium method described above can give structural dimensions down to 1 or 2 microns but not to dimensions below this.

Smaller surface features than this lead to interesting effects. One known effect is the creation of images from complex diffraction patterns. Although sometimes referred to as holograms, these images are not strictly holographic. Rather, variations in the number, density, length, direction, depth and shape, of lines cut into the surface of a work-piece can lead to very complex interference patterns that appear to be images. Such images may also display variations in colour.

In order to create complex diffraction patterns like this, the cut lines are sub-micron in width and it is not possible with conventional tooling methods to obtain this level of resolution within a deterministic structure directly on the surface of a forming tool.

The prior art surface structuring approaches possess a number of disadvantages. Eventually forming tools wear out and are either expensive or difficult to refurbish. Also, it is difficult and sometimes impossible to produce deterministic structures. It is especially difficult to produce very fine, sub-micron, deterministic structures within the coating on a forming tool. Furthermore, forming tools are generally used for single purposes, that is, with one kind of shape or surface structure in mind. They do not provide flexibility in the sense of it being easy and straightforward to change the surface of the forming tool.

It is an object of this invention to provide a new forming tool, one that can have its surface easily modified and one that can be produced with deterministic structures and very fine deterministic structures, the said surface features being transferable to a work-piece by any suitable forming method thereby giving the surface of the work-piece itself a fine, deterministic structure.

It is a further object of this invention to provide a new method of modifying the surface of a work-piece using a forming tool that itself has a structured surface.

It is a further object of the invention that the surface of the forming tool can be easily and inexpensively produced and eventually refurbished and to provide a method of preparing and refurbishing such forming tools.

Accordingly a first aspect of the invention is a forming tool comprising substrate and a metallic glass layer on at least the working face of the forming tool, characterised in that the metallic glass layer possesses a structured surface for the purpose of reproducing the structured surface of the metallic glass layer in the surface of a work-piece.

It will be readily appreciated that the metallic glass layer need not be directly adjacent to the working face of the forming tool and that other intermediate and functional layers may be incorporated, for example a compliant layer to accommodate differences in thermal expansion coefficients.

Metallic glasses are multi-component metallic alloys that, when cooled from a molten state at a fast enough rate, preferably retain an amorphous state when solid. Metallic glasses can also be slightly or partially crystallised when solid after cooling. These materials can be up to twice as strong as steel, have greater wear and corrosion resistance and have higher elasticity values than steel.

Metallic glasses suitable for the purpose herein described can be, for example, any one of the following group of general alloy systems: Au-Pb-Sb, Pd-Ni-P, La-Al-Ni, La-Al-Cu, La-Al-Ni-Cu, Mg-Cu-Y, Zr-Al-Ni-Cu, Zr-Ti-Cu-Ni-Al, Zr-Ti-Cu-Ni-Be, Zr-Ti-Nb-Cu-Ni-Be, Pd-Cu-Ni-P, Ni-Nb-Ta, Al-Co-Zr, Al-Ni-Ce-B, Al-Ni-Y-Co-B. These alloy systems are particularly useful because they can be cooled at slower rates than other metallic glasses yet still retain their amorphous state. One specific alloy that could be used is one containing, by weight percent, Zr 56.2, Ti 13.8, Nb 5, Cu7, Ni 5.5, Be 12.5. They can be cooled such that thickness of the metallic glass is of the order of 0.01 to 10 mm. This is important in this invention because the glass coating is on a substrate and the combined thermal mass means that extremely fast cooling rates are not always possible. In many situations the substrate itself can be used as an effective heat sink, either alone or in combination with other cooling means.

Where the intention is to make very fine deterministic structures the thickness of the metallic glass layer need not be very high. For example it could be a thin layer between 0.001 mm and 2 mm, in particular between 0.01 mm and 2 mm thick. Where the surface structure desired contains more prominent features then the metallic glass layer will preferably be thicker, between 0.5 mm and 30 mm, in particular between 0.5 mm and 10 mm thick. There is no need to have a large excess of glass because that would simply be a waste of material but there needs to be enough to enable the required structure to be formed within its surface. The lower thickness limit of the metallic glass is e.g. 0.001 mm, preferably 0.01 mm and more preferably 0.5 mm. The upper thickness limit of the metallic glass depends on the intended application but is for example not more than 30 mm, preferably 20 mm, more preferably 10 mm and even more preferably 5 mm.

The substrate could comprise any suitable shape typical of conventional forming tools that might be used in any of the forming methods previously mentioned. Also there is no particular requirement that the shape of the surface onto which the metallic glass is deposited to be of a certain kind. The metallic glass layer need not be deposited on the whole of the forming tool, merely on that face which comes into contact with the work-piece to be formed or modified, herein referred to as the working face. In other words, the working face is that face of the forming tool through which load is applied to the work-piece. The working face could be substantially planar or profiled, (in the sense that its shape face varies in at least two dimensions). Alternatively the shape of the working face may be at least a segment of the surface of a cylinder, as would be the case with a work roll for a metal rolling mill. In the latter case the substrate itself may be at least partly cylindrical or it could be a complete cylinder.

A particular advantage of the invention is that the structured surface of the metallic glass layer can be provided with a very fine deterministic structure. It is a preferred embodiment of the invention that the structured surface be deterministic and a more preferred embodiment that the deterministic structured surface contain features which are sub-micron in size.

A second aspect of the invention is a method of modifying the surface of a work-piece wherein at least one surface of the work-piece comes into contact with the structured surface of a forming tool at least once, the forming tool comprising a substrate and a metallic glass layer on at least the working face of the forming tool, characterised in that the metallic glass layer possesses a structured surface whereby the structured surface of the metallic glass layer reproduces in the surface of the work-piece.

The nature of the metallic glass layer in terms of its composition and thickness are typically the same as those described above in connection with the forming tool. Likewise, the structured surface can be stochastic in nature but it is preferred that it is deterministic and even more preferred that it contains features which are sub-micron in size.

Often forming operations of this nature take place in a number of repeat actions and therefore another embodiment of the invention is that this method involves a plurality of contacts between the work-piece and forming tool. This is often desirable because the transfer of the structural features from the surface of the forming tool to the work-piece is rarely perfect and more than one impression may be needed to generate the final desired surface on the work-piece.

In addition the transfer of the structure from the forming tool to the work-piece may take place under very low loading such that there is little or no reduction in the thickness of the work-piece. This is particularly useful in embossing operations.

A preferred embodiment involves the use of this method in the rolling of metal sheet where the forming tool is a work roll of a metal rolling mill. This embodiment is particularly suited to the rolling of aluminium and aluminium alloys.

A further aspect of the invention is a method of structuring the outer surface of a forming tool, the forming tool comprising a substrate and a metallic glass layer characterised by the steps of:
(a) heating at least the outer surface of the metallic glass layer to a temperature above its glass transition temperature,
(b) bringing the outer surface of the metallic glass layer into contact with the structured surface of a template for a period of time and under pressure such that the structured surface of the template is reproduced in the outer surface of the metallic glass layer to create a structured outer surface on the metallic glass layer,
(c) at least the structured outer surface of the metallic glass layer is cooled down at a rate sufficient to retain a mostly amorphous structure throughout the metallic glass layer,
(d) and the forming tool and the template are separated, the features of the structured surface of the template being retained within the structured outer surface of the metallic glass layer,

It has been surprisingly found that the surface of metallic glasses can be heated up until they are soft and can then be pressed against a template, the template possessing on its surface the structure or pattern desired in the surface of the metallic glass. After coming into contact with the template, at least the outer surface of the metallic glass layer is cooled and separated from the template. Of course the bulk of the metallic glass layer itself will also cool to some extent, it may even cool at a rate similar to the cooling rate of the outer surface. The cooling rate is sufficient such that the amorphous state is retained throughout the metallic glass. The surface structure of the template, which has been reproduced in the surface of the metallic glass, is retained after cooling in the outer surface of the metallic glass layer. Where the surface structure of the template contains large impressions or indentations then some of the bulk of the metallic glass layer may also be deformed so that the metallic glass layer as a whole displays the same external profile. A forming tool with a metallic glass layer thus formed is then used to modify the surface of the chosen work-piece.

The template could be made from conventional materials such as copper, aluminium or steel but is preferably made from a material that is able to withstand the high temperatures and pressures involved. Therefore steel or nickel templates are preferred. In order to facilitate the release of the template from the metallic glass at the relatively high temperatures in question a release agent may be applied to the surface of the template prior to coming into contact with the softened metallic glass.

The metallic glass, after coming into contact with the template, has to be cooled down at a rate fast enough to ensure that the metallic glass retains its amorphous structure below the glass transition temperature. The cooling rate necessary for this will depend on the metallic glass used but will normally be >10°C/sec, preferably >100°C/sec, more preferably >200°C/sec. In some situations, for example where the metallic glass has a large critical casting thickness, or the thickness of the metallic glass is small, effective cooling can be achieved by using forced gas, as for example air but in other situations it may be necessary to use means such as a fluid, as for example water or a water spray to bring about faster cooling rates. Other cooling means are solid materials having a high thermal conductivity such as metals, preferably copper and the like.

The invention will now be illustrated by reference to the following examples.

Figure 1 is a schematic of a simple forming tool incorporating the metallic glass layer on its working face and a method of using the forming tool.

Figure 2 is a schematic of one method of structuring the outer surface of a metallic glass layer, in this case in connection with a work roll suitable for metal sheet rolling.

Figure 3 is an image of the structured surface of a template made of tungsten carbide used to create a structured surface in the surface of a piece of metallic glass.

Figure 4 is an image of the structured surface of the metallic glass produced after coming into contact with the structured template having the surface of Figure 3.

Figure 5 is an image of the surface of aluminium sheet formed after a flat aluminium sheet was pressed against the structured surface of the metallic glass.

In Figure 1, the forming tool (10) is made up of a substrate (11) and a metallic glass layer (13) on the working face (12) of the forming tool. The metallic glass layer has a structured surface (14). Under load, as shown by the arrow, the structured surface (14) is brought into contact with the surface (16) of the work-piece (15). In this example the work-piece (15) is supported on a base plate (17). With a sufficient load applied, the surface of the work-piece will be modified and the features of the structured surface of the forming tool will be reproduced in the surface of the work-piece. It will be readily appreciated that the profile of the working face, as shown by line A-A', need not be flat but could be profiled. Likewise the base plate (17) could be a shaped die to match the profile of the forming tool. As mentioned above, the surface of the work-piece may not be an exact replica of the structured surface of the forming tool and the forming action may be repeated a number of times, preferably 2, 3, 4 times or more, to ensure the final surface of the work-piece has the desired features.

In Figure 2 the forming tool (20) is in the form of a cylindrical work roll intended for further use in rolling metal sheet. The forming tool (20) comprises a cylindrical substrate (21) and a metallic glass layer (23) on the working face (22). In this embodiment the cylindrical forming tool is made to rotate and the outer surface (27a) at least of the metallic glass layer (23) is heated up by a suitable heater (24) to a temperature above the glass transition temperature of the metallic glass. Above the glass transition temperature the metallic glass layer, or at least its outer surface, is soft enough to be modified. The outer surface of the metallic glass layer is then brought into contact with a template (25). In this example the template is a nickel shim which possesses, at least on one face a structured surface (26), either stochastic or deterministic in nature. The structured surface (26) of the template is brought into contact with the soft outer surface of the metallic glass and pressure is applied with the aid of two drive rolls (28a and 28b). After contact the outer surface of the metallic glass layer is modified and is converted into a structured outer surface (27b) of the metallic glass layer. In order to preserve the newly structured outer surface of the metallic glass layer at least the structured outer surface of the metallic glass layer is cooled down at a rate sufficiently fast to retain an amorphous structure throughout the metallic glass layer. It is possible, as well, to cool down the metallic glass layer from the working face side and the outer surface. This method may be a continuous system and it is within the bounds of the invention that the surface modification method herein described may be repeated a number of times. If this is the case in this embodiment, the structured outer surface (27b) of the metallic glass layer may, on further rotation, be heated up as before and structured a second or third time by contact with the template. In this way, if the initial structured surface of the metallic glass layer is not deemed to be adequate for its intended purpose it can be further improved and refined.

In another embodiment the template may be fed round another series of rolls (not illustrated) back to the start in a continuous loop. In such a case the length of template may be carefully controlled to correspond to the diameter of the substrate cylindrical work roll, especially if the structure to be created is deterministic. The diameter of the cylindrical work roll is not critical. The forming tool and the template are separated in the region of point B. In some circumstances, for example when the glass transition temperature is high and there is a danger of the metallic glass and the template sticking together, a suitable release agent is applied to the structured surface of the template to make separation easier.

A typical heater would be an induction heater, heating by conduction or a convection heater such as an infrared heater but may also include for example contact heaters, flame heaters, Joule effect heaters, hot gas heaters, or any other adequate heating device.

The structured surface of the metallic glass layer and the metallic glass layer itself may start to cool down even as the template and forming tool are in contact, i.e. before they are separated in this case. The cooling can be effected by the bulk of the substrate itself acting as a heat sink, which can be improved with the use of a cooling system built into the substrate. It is common for cylindrical work rolls to contain a chilled fluid such as a water system and this can be used to help provide the fast cooling required. Cooling can be further enhanced by forced gas, for example air cooling, applied on the exit side in the vicinity of the area marked B.

The forming tool with its surface structured according to the method illustrated by Figure 2 can then be used in a conventional rolling mill to modify the structure of work-pieces such as steel, aluminium and copper sheet.

To demonstrate that it is possible to replicate a structured surface from a template onto a surface of metallic glass and then onto a metallic work-piece a piece of metallic glass with a composition, (in weight %), Pd 40%, Ni 20%, Cu 30% and P 10%, possessing a glass transition temperature of 307°C and a recrystallization temperature of 407°C was selected. A tungsten carbide template with a structured surface was used to structure the surface of the metallic glass layer by heating both the template and the piece of metallic glass to a temperature of 380°C and bringing them into contact under a ramped pressure of 4 to 20MPa increasing over a duration of one second. The template and metallic glass were then separated and the metallic glass piece was allowed to cool down. The surface of the template consisted of a series of peaks and troughs with a depth to height value of around 9µm.

The topography of the template is shown in Figure 3 and the topography formed in the metallic glass surface is shown in Figure 4. The peak to trough distance in the metallic glass layer was also around 9µm.

The metallic glass piece with the structured layer on one surface was then used to stamp aluminium sheet. The aluminium sheet had a composition Fe 0.2%, Si 0.1%, balance aluminium and impurities. At room temperature the metallic glass piece was pressed against the aluminium sheet using a pressure of 70MPa for one second with the structured surface of the metallic glass piece facing the aluminium strip. Figure 5 shows the topography of the surface of the aluminium sheet thus formed. Comparison with Figure 3 shows that the structure from the template was very effectively transferred by the metallic glass piece into the surface of the aluminium sheet, albeit with a slightly smaller difference in height between peaks and troughs, the height being around 7µm.

The tool and processes according to the invention offer a range of advantages. They allow a greater degree of reproducibility from one manufacturing plant to another. For example, two similar forming tools can be created in different locations because the same template can be used to produce almost identical tools. The template can be moved from one manufacturing plant to another and the working surface of the forming tool can be structured in exactly the same way at different locations. This will ensure consistency in the final form of the work-pieces being manufactured. Further, the very first structured forming tool can be used as a master tool and it can be used to generate a number of templates for use in other locations, again making production consistent from one manufacturing facility to another.

The processes described enable the creation of very small and deterministic surface features in a simple and effective way. This will have a wide range of benefits in many forming industries and has the potential to eliminate some subsequent processing steps. For example, if the forming operation also enables marking of the work-piece, a subsequent marking or printing step using another process can be dispensed with. This provides the user with the means to individualise their manufactured products more easily and distinctively.

The tool and processes according to the invention facilitate longer forming tool life. The properties of the metallic glass layer are well suited to prolonging tool life. Their high elastic strain limits, combined with high strength and high toughness means that the metallic glass layer remains in the fully elastic range during forming operations, far away from the metallic glass yield strength. As a result the structured surface of the metallic glass layer retains its integrity for much longer than other forming tool protective layers.

Furthermore, by re-heating the metallic glass surface layer and refurbishing the structure in exactly the same way as it had previously been formed, the life of the forming tool and its working surface can be further extended and any deterioration in the quality of the surface structure can be easily corrected.

In addition, the same conditioning and refurbishing process allows the manufacturer to change the structure of the working surface with a minimum of effort. This provides enhanced flexibility in design and production scheduling.

A forming tool according to the invention and the method of modifying the surfaces of work-pieces according to the invention may be used, by way of example, in the production of sheet and shaped parts for automotive use, the production of lithographic sheet, the production of coins and badges and the production of reflector sheet.

## Claims

1. A forming tool (10, 20) comprising a substrate (11, 21) and a metallic glass layer (13, 23) on at least the working face (12, 22) of the forming tool (10, 20), **characterised in that** the metallic glass layer (13, 23) possesses a structured surface (14, 27b) for the purpose of reproducing the structured surface (14, 27b) of the metallic glass layer in the surface (16) of a work-piece (15).

2. A forming tool as claimed in claims 1 **characterised in that** there is at least one other functional layer between the working face of the forming tool and the metallic glass layer.

3. A forming tool as claimed in claims 1 and 2 **characterised in that** the metallic glass layer has an upper limit of its thickness of 30 mm, preferably 10 mm and a lower limit of 1 µm, preferably 10 µm.

4. A forming tool as claimed in claim 3 **characterised in that** the metallic glass layer has a lower limit of its thickness of 0.5 mm.

5. A forming tool as claimed in claim 3 **characterised in that** the metallic glass layer has an upper limit of its thickness of 8 mm.

6. A forming tool as claimed in claim 3 **characterised in that** the metallic glass layer has an upper limit of its thickness of 5 mm.

7. A forming tool as claimed in claim 1 and 2 **characterised in that** the metallic glass layer has a thickness between 10 µm and 10 mm.

8. A forming tool as claimed in claims 1 to 7 **characterised in that** the working face of the substrate is substantially planar.

9. A forming tool as claimed in claim 1 to 7 **characterised in that** the working face of the substrate is profiled.

10. A forming tool as claimed in claim 1 to 7 **characterised in that** the shape of the forming tool is at least partly cylindrical.

11. A forming tool as claimed in claim 10 **characterised in that** the forming tool is a cylindrical work roll.

12. A forming tool as claimed in claims 1 to 11 **characterised in that** the structured surface of the metallic glass is deterministic.

13. A forming tool as claimed in claim 12 **characterised in that** the deterministic structure comprises features having dimensions below 1 µm in size.

14. A forming tool as claimed in claims 1 to 13 **characterised in that** the composition of the metallic glass layer is an alloy from a group consisting of the following alloy systems: Au-Pb-Sb, Pd-Ni-P, La-Al-Ni, La-Al-Cu, La-Al-Ni-Cu, Mg-Cu-Y, Zr-Al-Ni-Cu, Zr-Ti-Cu-Ni-Al, Zr-Ti-Cu-Ni-Be, Zr-Ti-Nb-Cu-Ni-Be, Pd-Cu-Ni-P, Ni-Nb-Ta, Al-Co-Zr, Al-Ni-Ce-B, Al-Ni-Y-Co-B.

15. A method of modifying the surface (16) of a work-piece (15) wherein at least one surface (16) of the work-piece (15) comes into contact with the structured surface (14) of a forming tool (10) at least once, the forming tool (10) comprising a substrate (11) and a metallic glass layer (13) on at least the working face (12) of the forming tool (10), **characterised in that** the metallic glass layer (13) possesses a structured surface (14) whereby the structured surface (14) of the metallic glass layer (13) reproduces in the surface (16) of the work-piece (15).

16. A method as claimed in claim 15 **characterised in that** there is a plurality of contacts, preferably 2, 3 or 4, between the work-piece and the forming tool.

17. A method as claimed in claim 15 and 16 **characterised in that** the forming tool is a work roll of a metal rolling mill.

18. A method as claimed in claims 15 to 17 **characterised in that** the work-piece is at least a part of a metal sheet.

19. A method as claimed in claims 15 to 18 **characterised in that** the work-piece is aluminium or an aluminium alloy.

20. A method as claimed in claims 15 to 19 **characterised in that** the pressure applied during forming provides essentially no reduction in the thickness of the work-piece.

21. A method of structuring the outer surface (27a) of a forming tool (20), the forming tool (20) comprising a substrate (21) and a metallic glass layer (23) **characterised by** the steps of:
(a) heating at least the outer surface (27a) of the metallic glass layer (23) to a temperature above its glass transition temperature,
(b) bringing the outer surface (27a) of the metallic glass layer (23) into contact with the structured surface (26) of a template (25) for a period of time and under pressure such that the shaped surface (26) is reproduced in the structured outer surface (27b) of the metallic glass layer (23),
(c) at least the structured outer surface (27b) of the metallic glass layer (23) is cooled down at a rate sufficient to retain a mostly amorphous structure throughout the metallic glass layer (23),
(d) and the forming tool (20) and the template (25) are separated, the features of the structured surface (26) of the template (25) being retained within the structured outer surface (27b) of the metallic glass layer (23).

22. A method as claimed in claim 21 **characterised in that** the steps (a) to (d) are repeated at least once.

23. A method as claimed in claims 21 and 22 **characterised in that** the heating step is carried out using an induction heater.

24. A method as claimed in claim 21 and 22 **characterised in that** the heating step is carried out using a convection heater.

25. A method as claimed in claims 21 to 24 **characterised in that** cooling of the metallic glass layer is assisted by a cooling system within the substrate.

26. A method as claimed in claims 21 to 25 **characterised in that** the template is a nickel shim.

27. A method as claimed in claims 21 to 26 **characterised in that** the forming tool is a cylindrical work roll for use in a metal rolling mill.

28. A method as claimed in claims 21 to 27 **characterised in that** a release agent is deposited onto the shaped surface of the template.

## Patentansprüche

1. Formwerkzeug (10, 20), **dadurch gekennzeichnet, dass** es ein Substrat (11, 21) und eine Schicht aus metallischem Glas (13, 23) zumindest auf der Arbeitsfläche (12, 22) des Formwerkzeugs (10, 20) umfasst und die Schicht aus metallischem Glas (13, 23) eine strukturierte Oberfläche (14, 27b) zum Zweck des Reproduzierens der strukturierten Oberfläche (14, 27b) der Schicht aus metallischem Glas in der Oberfläche (16) eines Werkstücks (15) besitzt.

2. Formwerkzeug nach Anspruch 1, **dadurch gekennzeichnet, dass** es zwischen der Arbeitsfläche des Formwerkzeugs und der Schicht aus metallischem Glas wenigstens eine weitere funktionelle Schicht gibt.

3. Verfahren nach Anspruch 1 und 2, **dadurch gekennzeichnet, dass** die Schicht aus metallischem Glas eine Dicke mit einer Obergrenze von 30 mm, vorzugsweise 10 mm, und einer Untergrenze von 1 µm, vorzugsweise 10 µm, hat.

4. Verfahren nach Anspruch 3, **dadurch gekennzeichnet, dass** die Schicht aus metallischem Glas eine Dicke mit einer Untergrenze von 0,5 mm hat.

5. Verfahren nach Anspruch 3, **dadurch gekennzeichnet, dass** die Schicht aus metallischem Glas eine Dicke mit einer Obergrenze von 8 mm hat.

6. Verfahren nach Anspruch 3, **dadurch gekennzeichnet, dass** die Schicht aus metallischem Glas eine Dicke mit einer Obergrenze von 5 mm hat.

7. Verfahren nach Anspruch 1 und 2, **dadurch gekennzeichnet, dass** die Schicht aus metallischem Glas eine Dicke zwischen 10 µm und 10 mm hat.

8. Formwerkzeug nach einem der Ansprüche 1 bis 7, **dadurch gekennzeichnet, dass** die Arbeitsfläche des Substrats im Wesentlichen eben ist.

9. Formwerkzeug nach einem der Ansprüche 1 bis 7, **dadurch gekennzeichnet, dass** die Arbeitsfläche des Substrat mit einem Profil versehen ist.

10. Formwerkzeug nach einem der Ansprüche 1 bis 7, **dadurch gekennzeichnet, dass** die Gestalt des Formwerkzeugs wenigstens teilweise zylindrisch ist.

11. Formwerkzeug nach Anspruch 10, **dadurch gekennzeichnet, dass** das Formwerkzeug eine zylindrische Arbeitswalze ist.

12. Formwerkzeug nach einem der Ansprüche 1 bis 11, **dadurch gekennzeichnet, dass** die strukturierte Oberfläche des metallischen Glases deterministisch ist.

13. Formwerkzeug nach Anspruch 12, **dadurch gekennzeichnet, dass** die deterministische Struktur Merkmale umfasst, die Dimensionen in einer Größe unter 1 µm haben.

14. Formwerkzeug nach einem der Ansprüche 1 bis 13, **dadurch gekennzeichnet, dass** die Zusammensetzung der Schicht aus metallischem Glas eine Legierung aus einer Gruppe bestehend aus den folgenden Legierungssystemen ist: Au-Pb-Sb, Pd-Ni-P, La-Al-Ni, La-Al-Cu, La-Al-Ni-Cu, Mg-Cu-Y, Zr-Al-Ni-Cu, Zr-Ti-Cu-Ni-Al, Zr-Ti-Cu-Ni-Be, Zr-Ti-Nb-Cu-Ni-Be, Pd-Cu-Ni-P, Ni-Nb-Ta, Al-Co-Zr, Al-Ni-Ce-B, Al-Ni-Y-Co-B.

15. Verfahren zum Modifizieren der Oberfläche (16) eines Werkstücks (15), bei dem wenigstens eine Oberfläche (16) des Werkstücks (15) wenigstens einmal mit der strukturierten Oberfläche (14) eines Formwerkzeugs (10) in Kontakt kommt, **dadurch gekennzeichnet, dass** das Formwerkzeug (10) aus einem Substrat (11) und einer Schicht aus metallischem Glas (13) wenigstens auf der Arbeitsfläche (12) des Formwerkzeugs (10) besteht und die Schicht aus metallischem Glas (13) eine strukturierte Oberfläche (14) besitzt, wodurch die strukturierte Oberfläche (14) der Schicht aus metallischem Glas (13) in der Oberfläche (16) des Werkstücks (15) reproduziert wird.

16. Verfahren nach Anspruch 15, **dadurch gekennzeichnet, dass** sich zwischen dem Werkstück und dem Formwerkzeug mehrere Kontakte, vorzugsweise 2, 3 oder 4, befinden.

17. Verfahren nach Anspruch 15 und 16, **dadurch gekennzeichnet, dass** das Formwerkzeug eine Arbeitswalze eines Metallwalzwerks ist.

18. Verfahren nach einem der Ansprüche 15 bis 17, **dadurch gekennzeichnet, dass** das Werkstück wenigstens ein Teil eines Blechs ist.

19. Verfahren nach einem der Ansprüche 15 bis 18, **dadurch gekennzeichnet, dass** das Werkstück Aluminum oder eine Aluminiumlegierung ist.

20. Verfahren nach einem der Ansprüche 15 bis 19, **dadurch gekennzeichnet, dass** der während des Formens angewendete Druck im Wesentlichen keine Verringerung der Dicke des Werkstücks bewirkt.

21. Verfahren zum Strukturieren der Außenfläche (27a) eines Formwerkzeugs (20), **dadurch gekennzeichnet, dass** das Formwerkzeug (20) ein Substrat (21) und eine Schicht aus metallischem Glas (23) umfasst, umfassend die folgenden Schritte:
a) Erwärmen wenigstens der Außenfläche (27a) der Schicht aus metallischem Glas (23) auf eine Temperatur über ihrer Glasübergangstemperatur,
b) Inkontaktbringen der Außenfläche (27a) der Schicht aus metallischem Glas (23) mit der strukturierten Oberfläche (26) einer Schablone (25) für eine Zeitspanne und unter Druck, so dass die formgestaltete Oberfläche (26) in der strukturierten Außenfläche (27b) der Schicht aus metallischem Glas (23) reproduziert wird,
c) Abkühlen von wenigstens der strukturierten Außenfläche (27b) der Schicht aus metallischem Glas (23) mit einem Tempo, das ausreicht, um in der Schicht aus metallischem Glas (23) weitgehend durchgehend ein amorphes Gefüge beizubehalten,
d) und Trennen des Formwerkzeugs (20) und der Schablone (25), wobei die Merkmale der strukturierten Oberfläche (26) der Schablone (25) in der strukturierten Außenfläche (27b) der Schicht aus metallischem Glas (23) beibehalten werden.

22. Verfahren nach Anspruch 21, **dadurch gekennzeichnet, dass** die Schritte a) bis d) wenigstens einmal wiederholt werden.

23. Verfahren nach Anspruch 21 und 22, **dadurch gekennzeichnet, dass** der Erwärmungsschritt mit einer Induktionsheizvorrichtung durchgeführt wird.

24. Verfahren nach Anspruch 21 und 22, **dadurch gekennzeichnet, dass** der Erwärmungsschritt mit einer Konvektionsheizvorrichtung durchgeführt wird.

25. Verfahren nach einem der Ansprüche 21 bis 24, **dadurch gekennzeichnet, dass** das Kühlen der metallischen Glasschicht durch ein Kühlsystem in dem Substrat unterstützt wird.

26. Verfahren nach einem der Ansprüche 21 bis 25, **dadurch gekennzeichnet, dass** die Schablone eine Nickelbeilage ist.

27. Verfahren nach einem der Ansprüche 21 bis 26, **dadurch gekennzeichnet, dass** das Formwerkzeug eine zylindrische Arbeitswalze zur Verwendung in einem Metallwalzwerk ist.

28. Verfahren nach einem der Ansprüche 21 bis 27, **dadurch gekennzeichnet, dass** ein Trennmittel auf die formgestaltete Oberfläche der Schablone aufgebracht wird.

## Revendications

1. Outil de formage (10, 20) **caractérisé en ce qu'**il comprend un substrat (11, 21) et une couche de verre métallique (13, 23) sur au moins la face de travail (12, 22) de l'outil de formage (10, 20) et la couche de verre métallique (13, 23) possède une surface structurée (14, 27b) afin de reproduire 1a surface structurée (14, 27b) de 1a couche de verre métallique dans la surface (16) d'une pièce (15).

2. Outil de formage selon la revendication 1, **caractérisé en ce que** l'on trouve au moins une autre couche fonctionnelle entre la face de travail de l'outil de formage et la couche de verre métallique.

3. Procédé selon les revendications 1 et 2, **caractérisé en ce que** la couche de verre métallique a une limite supérieure de son épaisseur de 30 mm, de préférence 10 mm et une limite inférieure de 1 µm, de préférence 10 µm.

4. Procédé selon la revendication 3, **caractérisé en ce que** la couche de verre métallique a une limite inférieure de son épaisseur de 0,5 mm.

5. Procédé selon la revendication 3, **caractérisé en ce que** la couche de verre métallique a une limite supérieure de son épaisseur de 8 mm.

6. Procédé selon la revendication 3, **caractérisé en ce que** la couche de verre métallique a une limite supérieure de son épaisseur de 5 mm.

7. Procédé selon les revendications 1 et 2, **caractérisé en ce que** la couche de verre métallique a une épaisseur comprise entre 10 µm et 10 mm.

8. Outil de formage selon les revendications 1 à 7, **caractérisé en ce que** la face de travail du substrat est sensiblement plane.

9. Outil de formage selon les revendications 1 à 7, **caractérisé en ce que** la face de travail du substrat est profilée.

10. Outil de formage selon les revendications 1 à 7, **caractérisé en ce que** la forme de l'outil de formage est au moins partiellement cylindrique.

11. Outil de formage selon la revendication 10, **caractérisé en ce que** l'outil de formage est un cylindre de travail cylindrique.

12. Outil de formage selon la revendication 1 à 11, **caractérisé en ce que** la surface structurée du verre métallique est déterministique.

13. Outil de formage selon la revendication 12, **caractérisé en ce que** la structure déterministique comprend des caractéristiques ayant des dimensions inférieures à 1 µm du point de vue de la taille.

14. Outil de formage selon les revendications 1 à 13, **caractérisé en ce que** la composition de la couche de verre métallique est un alliage d'un groupe se composant des systèmes d'alliage suivants : Au-Pb-Sb, Pd-Ni-P, La-Al-Ni, La-Al-Cu, La-Al-Ni-Cu, Mg-Cu-Y, Zr-Al-Ni-Cu, Zr-Ti-Cu-Ni-Al, Zr-Ti-Cu-Ni-Be, Zr-Ti-Nb-Cu-Ni-Be, Pd-Cu-Ni-P, Ni-Nb-Ta, Al-Co-Zr, Al-Ni-Ce-B, Al-Ni-Y-Co-B.

15. Procédé pour modifier la surface (16) d'une pièce (15) dans lequel au moins une surface (16) de la pièce (15) vient en contact avec la surface structurée (14) d'un outil de formage (10) au moins une fois, **caractérisé en ce que** l'outil de formage (10) est composé d'un substrat (11) et d'une couche de verre métallique (13) sur au moins la face de travail (12) de l'outil de formage (10) et la couche de verre métallique (13) possède une surface structurée (14) moyennant quoi la surface structurée (14) de la couche de verre métallique (13) reproduit la surface (16) de la pièce (15).

16. Procédé selon la revendication 15, **caractérisé en ce que** l'on trouve une pluralité de contacts, de préférence 2, 3 ou 4, entre la pièce et l'outil de formage.

17. Procédé selon les revendications 15 et 16, **caractérisé en ce que** l'outil de formage est un cylindre de travail d'un laminoir à métal.

18. Procédé selon les revendications 15 à 17, **caractérisé en ce que** la pièce fait au moins partie d'une tôle.

19. Procédé selon les revendications 15 à 18, **caractérisé en ce que** la pièce est en aluminium ou un alliage d'aluminium.

20. Procédé selon les revendications 15 à 19, **caractérisé en ce que** la pression appliquée pendant le formage ne fournit sensiblement pas de réduction de l'épaisseur de la pièce.

21. Procédé pour structurer la surface externe (27a) d'un outil de formage (20) **caractérisé en ce que** l'outil de formage (20) comprend un substrat (21) et une couche de verre métallique (23) comprenant les étapes consistant à :
(a) chauffer au moins la surface externe (27a) de la couche de verre métallique (23) à une température supérieure à sa température de transition vitreuse,
(b) amener la surface externe (27a) de la couche de verre métallique (23) en contact avec la surface structurée (26) d'un gabarit (25) pendant une période de temps et sous pression de sorte que la surface formée (26) est reproduite dans la surface externe structurée (27b) de la couche de verre métallique (23),
(c) au moins la surface externe structurée (27b) de la couche de verre métallique (23) est refroidie à une vitesse suffisante pour conserver une structure principalement amorphe dans toute la couche de verre métallique (23),
(d) et l'outil de formage (20) et le gabarit (25) sont séparés, les caractéristiques de la surface structurée (26) du gabarit (25) étant retenues à l'intérieur de la surface externe structurée (27b) de la couche de verre métallique (23).

22. Procédé selon la revendication 21, **caractérisé en ce que** les étapes (a) à (d) sont répétées au moins une fois.

23. Procédé selon les revendications 21 et 22, **caractérisé en ce que** l'étape de chauffage est réalisée en utilisant un dispositif de chauffage à induction.

24. Procédé selon les revendications 21 et 22, **caractérisé en ce que** l'étape de chauffage est réalisée en utilisant un dispositif de chauffage à convection.

25. Procédé selon les revendications 21 à 24, **caractérisé en ce que** le refroidissement de la couche de verre métallique est assisté par un système de refroidissement à l'intérieur du substrat.

26. Procédé selon les revendications 21 à 25, **caractérisé en ce que** le gabarit est une cale de réglage en nickel.

27. Procédé selon les revendications 21 à 26, **caractérisé en ce que** l'outil de formage est un cylindre de travail cylindrique destiné à être utilisé dans un laminoir à métal.

28. Procédé selon les revendications 21 à 27, **caractérisé en ce qu'**un agent de démoulage est déposé sur la surface formée du gabarit.
